

(No Model.)

H. ANDERSON.

PILE COVERING.

No. 366,444.

Patented July 12, 1887.

FIG. 1.



FIG. 2.



Witnesses

Leon C. Ballot

Ferdinand Imhors  
Charles P. Compton

Inventor:

Henry Anderson  
By his Atty.

Alphonse O. Smith

# UNITED STATES PATENT OFFICE.

HENRY ANDERSON, OF OAKLAND, CALIFORNIA, ASSIGNOR OF PART TO  
HENRY T. COMPTON AND JOHN MILTON KILE, BOTH OF SAME PLACE,  
AND ALEXANDER T. VOGELSANG, OF SAN FRANCISCO, CALIFORNIA.

## PILE-COVERING.

SPECIFICATION forming part of Letters Patent No. 366,444, dated July 12, 1887.

Application filed February 11, 1887. Serial No. 227,347. (No model.)

*To all whom it may concern:*

Be it known that I, HENRY ANDERSON, a citizen of the United States of America, and a resident of the city of Oakland, Alameda county, State of California, have invented new and useful Improvements in Pile-Covering, of which the following is a full, clear, and exact description, referring to the accompanying drawings.

10 The object of my invention is to provide suitable means for the protection of piles from the ravages of the terredo, lemnoria, or other marine insects.

15 Figure 1 shows an elevation of a pile and of my improved pile-covering. Fig. 2 shows a cross-section through the pile and my pile-covering.

In constructing my improved pile I begin by stripping a suitable portion of the bark from 20 the pile A. I then proceed to paint the uncovered section of the pile with a coating of tar, B, or other suitable paint. After the tar is painted I proceed to cover that section with a thick layer or cover of asphalt, C. Over 25 the asphalt I place a covering of sheet-lead, D, which I prefer to secure by suitable means, and as further security for fastening the sheet-lead, and to prevent injury to the lead covering by the rubbing or concussion of a vessel 30 or other material, I cover the sheet-lead by

wrapping metallic wire or strips E around the sheet-lead and secure the wire or strips E in a suitable manner by means of nails, screws, or solder to the lead covering and the pile, thus obviating the uncovering of the wire from 35 the pile and lead covering if by any cause whatsoever any section of the wire is severed or broken.

I do not confine myself to the use of lead as a covering material, as I may find it desirable 40 to construct my improved pile-covering without a covering of sheet-lead.

Having thus fully described my invention, what I claim, and desire to secure by Letters Patent, is—

1. As a pile-covering and applied to the bare wood of pile A, a coating of tar or paint, B, a covering of asphalt, C, sheet-lead D, metallic wire or strips E, substantially as and for the purpose set forth. 45

2. As a pile-covering and applied to the bare wood of pile A, a coating of tar or paint, B, a covering of asphalt, C, metallic wire or strips E, substantially as and for the purpose set forth. 50

HENRY ANDERSON. [L. s.]

Witnesses:

FERDINAND IMHORST,  
ALPHONSO B. SMITH,  
CHARLES F. GOMPERTZ.